# EUROPEAN PATENT SPECIFICATION

(11) **EP 1 425 453 B1**
(45) Date of publication and mention of the grant of the patent: **28.05.2008**
(21) Application number: 02787135.9
(22) Date of filing: 17.07.2002
(51) Int. Cl.: D04H 1/42, A41D 31/00

(54) **FLAMEPROOF YARNS AND FABRICS, THEIR PREPARATION AND USE FOR THE MANUFACTURING OF FLAMEPROOF, HEAT RESISTANT, AND INSULATING PRODUCTS**
SCHWERENTFLAMMBARE GARNE UND TEXTILE FLÄCHENGEBILDE, DEREN HERSTELLUNG UND VERWENDUNG ZUR HERSTELLUNG VON SCHWERENTFLAMMBAREN, HITZEBESTÄNDIGEN UND ISOLIERENDEN PRODUKTEN
FILS ET TOILES IGNIFUGES, LEUR PRODUCTION ET LEUR UTILISATION POUR LA REALISATION DE PRODUITS IGNIFUGES, RESISTANTS A LA CHALEUR, ET ISOLANTS

(30) Priority: 18.07.2001 IT FI20010136
(43) Date of publication of application: 09.06.2004
(73) Proprietor: EOS S.R.L., I-20049 Concorezzo (IT)
(72) Inventor: MONTINI, Leonardo, I-59100 Prato (IT)
(74) Representative: Gervasi, Gemma
(86) International application number: PCT/EP2002/007950
(87) International publication number: WO 2003/008689

(56) References cited:
- US-A- 4 600 572
- US-A- 4 865 906
- US-A- 4 987 664
- US-A- 6 021 523
- US-B1- 6 287 686
- DATABASE WPI Section Ch, Week 199018 Derwent Publications Ltd., London, GB; Class A14, AN 1990-136188 XP002215133 & JP 02 084526 A (ASAHI CHEM IND CO LTD), 26 March 1990 (1990-03-26)

## Description

### Field of the invention

The present invention relates to yarns and fabrics that present simultaneously high flameproof, heat resistant, and insulating characteristics, to their manufacturing process, and to their use for the manufacturing of flameproof, heat resistant, and insulating products.

### State of the art

As known in various activities, and in particular those relating to safety, it is essential to have products provided with fireproof properties, that allow the user to operate in environments having extremely high temperatures and in the presence fires (as for example in fire-fighting operations).

Excluding fabrics that contain asbestos, for the well known toxicity of this material, for the manufacturing of fabrics suitable to the above mentioned purposes the meta-aramidic fibres, as for example NOMEX® (that give the fabric the desired fireproof property) and the aramidic and/or para-aramidic ones, like KEVLAR® (that give them resistance to cuts) have been suggested.

The fabrics manufactured with the above-mentioned fibres, even with their various advantages, nevertheless also present various disadvantages that make their use uncomfortable; in particular, the products manufactured with these fabrics have a significant permeability to heat (and thus, even if they are fireproof, do not allow the operator to be exposed for a long time to the heat source) and, in contact with flames, easily tend to melt or carbonize, and then to disintegrate. Moreover, these materials are difficult to be processed when they have to be manufactured (as, for example, in the manufacturing of fireproof garments).

It is therefore advisable to develop new materials that allow to overcome the above mentioned disadvantages.

### Abstract of the invention

The present invention relates to fabrics consisting of pre-anodized acrylic fibres.

### Detailed description of the invention

The present invention allows to overcome the above-mentioned problems, thanks to fabrics comprising the fibres as defined above.

According to the present invention, with pre-anodized acrylic fibres we mean the fibres having this name normally used in the textile field, as for example those manufactured by Ashai Chemicals (LASTAN®), Toho Rajon (PIROMEX®), SGL (PANOX®), and Zoltek (PYRON®), and their blends.

The fabrics according to the present invention can be prepared, for example, acording to the process related here following and subject too to this patent application.

In the process according to the invention the fibres, in flocks, are spun obtaining both single and twisted yarns, having a metric number (that is metres, in thousands, per 1 Kg) between 10 and 60.

The yarns are dried by heating them on hot rolls (calendering).

The yarns so obtained can then be used in the manufacturing operations according to the normal weaving techniques of fabrics having any type of weave, for example from plain weave to satin, in which the yarn can be both woven and warped.

Given the smoothness and versatility of the fabric obtained with the fibres processed as mentioned above, the fabrics according to the present invention find a very wide use, for example in the manufacturing of protective clothing for fire-fighting operations, and military, industrial, sports use, etc. Moreover, they can be used in the manufacturing of structures useful for the protection of materials and plants from fire, or the flameproof textile upholstery and accessories for furnishing public areas like cinemas, theatres, discotheques, seats, etc..

In particular, the fabrics comprising only pre-anodized fibres have an exceptional heat resistance, that make them particularly suited to the manufacture of insulating elements (for example panels for fire doors, carters for protecting engines or machine parts, insulating elements for boots and similar equipment, etc.). Among these fabrics the felt ones are specially preferred.

Among these fabrics the felt ones are specially preferred. Usually this type of fabric has a low resistance, and therefore its use is limited; this is specially true in the fire protection applications, because any tear in the fabric would compromise its function.

The felt according to the present invention is prepared, for example, according to the process hereinafter described which is also a subject of the present application.

The pre-anodized fibres, in flocks, are turned into veils through the carding process; these veils are then needle felted so as to obtain the desired uniformity and solidity in the finished product.

The product's solidity is a function of the number of veils, the number of needles per square metres used, and the number of beatings carried out in the needle felting process (the higher the number of veils, needles, and beatings, the more solid ans resistant the product will be).

The felts having an areal mass higher than 100 g/m² are specially preferred.

Preferred are felts obtained with a carding process in which at least 6 to 11 veils are created (preferably from 7 to 9 veils) per finished product; and a needle felting process in which at least 5.000 to 10.000 needles per m² are used. (preferably from 7.000 to 9.000 needles per m²) and at least from 400 to 800 beatings per minute (preferably from 600 to 800 beatings per minute).

Once this process is finished, finished felts having various thickness can be needle felted together, with the same number of needles and beatings previously specified; this so as to obtain new finished felts having a total number of veils, needles used, and beatings that are the sum of the veils, needles, and beatings of the original felts. This further improves the toughness and resistance of the finished product.

If preferred, to further improve the product's mechanical properties the felt, after being needle felted, can be quilted with a yarn, in more or less large stitches, containing 100% of pre-anodized acrylic fibres, or these pre-anodized acrylic fibres in a blend with aramidic, or metal-aramidic, or para-aramidic fibres; or with a yarn comprising 100% aramidic, or metal-aramidic, or para-aramidic fibres; or again, during the needle felting process a net made in a mechanically resistant material (for example a Kevlar^{®} net) that will make up a weave for the same felt can be added inside the felt.

According to a further aspect of the invention, the net can be applied on one of the felt surfaces through the usual lamination or sizing techniques.

The above-mentioned processes, that are an integral part of the invention, are targeted, and allow to obtain a resistance and a toughness currently not available in the state of the art.

The felts manufactured according to the invention, comprising 100% in pre-anodized acrylic fibres like PANOX^{®} and LASTAN^{®}, underwent some resistance tests that gave the following results:
Tension resistance, according to the UNI EN ISO 29073/93 part 3a regulation, of a felt having an areal mass equal to 108 g/mq

| | |
|---|---|
| Lengthwise | Average breaking force 27,4 N |
| | Average breaking force 2,79 Kg |
| | Breaking stretch 37 % |
| Transversal | Average breaking force 20,5 N |
| | Average breaking force 2,09 Kg |
| | Breaking stretch 46,5 % |

Tension resistance, according to the UNI EN ISO 29073/93 part 3a regulation, of a felt having an areal mass equal to 206 g/mq

| | |
|---|---|
| Lengthwise | Average breaking force 44,6 N |
| | Average breaking force 4,55 Kg |
| | Breaking stretch 50 % |
| Transversal | Average breaking force 56,6 N |
| | Average breaking force 5,77 Kg |
| | Breaking stretch 31,5 % |

Moreover, oxy-hydrogen flame resistance tests have been carried out, to verify the drilling times of that same flame on a felt having an areal mass of 108 g/m² (100% pre-anodized acrylic fibres of the PANOX^{®} tipe), with an average thickness of 1,62 mm, at a distance of 15 cm from the nozzle of the oxyacetylene burner and a 800° C temperature.

The drilling time has been higher than 3 minutes, and the temperature at the opposite side, at 3 cm from the felt, before the drilling, never exceeded 50° C.

This behaviour makes the use of felts manufactured with this technique available as stuffing both for furniture and clothing use; up to now this was not possible with the said materials, due to their low resistance.

If necessary, the fabric according to the present invention can be laminated, sized, spread, and quilted with any other type of fabric to give the garment the desired characteristics.

## Claims

1. Felts comprising overlapping veils needle felted together consisiting of pre-anodised acrylic fibres.

2. Felts according to claim 1, having an areal mass higher than 100 g/m².

3. Felt according to claim 1, in which the number of veils is between 6 and 11.

4. Felt according to claim 3, in which the number of veils is between 7 and 9.

5. Felt according to claims 3 and 4 in which the veils undergo a carding and needle felting process, that foresees from 5.000 to 10.000 needles per m² and from 400 to 800 beatings per minute.

6. Felt according to claim 5 in which the needle felting process foresees the use of 7.000 - 9.000 needles per m² and 600 - 800 beatings per minute.

7. Felt according to the claims 1 - 6 in which the same felts are quilted in more or less large stitches.

8. Felt according to claim 7 in which the quilting foresees a yam comprising 100% of pre-anodised acrylic fibres.

9. Felt according to claim 7 in which the quilting foresees a yam comprising 100% of aramidic, meta-aramidic, or para-aramidic fibres.

10. Felt according to the claims 1 - 9 in which the said felt comprises a weave made of a net in mechanically resistant material.

11. Felt according to claim 10 in which the said weave is included inside the felt.

12. Felt according to claim 10 in which the said weave is applied on one of the felt surfaces through the usual lamination or sizing techniques.

13. Felt according to claim 1 comprising felts according to claims 2 - 5, needle felted together.

14. Process for the manufacturing of a felt according to the claims 1 - 6 in which pre-anodised acrylic fibres, in flocks, undergo the carding process and are transformed in overlapping veils that are then needle felted using 5.000 - 10.000 needles per m², carrying on 400 - 800 beatings per minute; and the felts so obtained are in tum needle felted together.

15. Process according to claim 14 in which the needle felting process is carried out using 7.000 - 9.000 needles and 600 - 800 beatings per minute.

16. Use of the felts according to the claims 1 - 13 for the manufacturing of insulating materials.

17. Use of the felts according to the claims 1 - 13 for the manufacturing of protective clothing for fire and heat, for the manufacturing of products for the protection of materials or plants from fire, of flameproof textile upholstery and accessories for furnishing public areas.

18. Insulating materials made of, or comprising, felts according to the claims 1 - 13.

19. Fireproof and heat resistant garments, products useful for protecting materials or plants from fire, flameproof textile upholstery and accessories for furnishing public areas, insulating materials made of, or comprising, felts according to claims 1 - 13.

20. Felts according to the claims 1 - 13 in which the pre-anodised acrylic fibre is LASTAN^{®} PIROMEX^{®}, PANOX^{®}, PYRON^{®} type, or their blend.

## Patentansprüche

1. Filze mit sich überlappenden Schleiern, die miteinander nadelgefilzt sind, bestehend aus voranodisierten Acrylfasern.

2. Filze nach Anspruch 1,
mit einer Flächenmasse von höher als 100 g/m².

3. Filz nach Anspruch 1,
wobei die Anzahl von Schleiern zwischen 6 und 11 liegt.

4. Filz nach Anspruch 3,
wobei die Anzahl von Schleiern zwischen 7 und 9 liegt.

5. Filz nach einem der Ansprüche 3 und 4,
wobei die Schleier einem Kardier- und Nadelfilzprozess ausgesetzt werden, der zwischen 5.000 bis 10.000 Nadeln pro m² und zwischen 400 bis 800 Schläge pro Minute vorsieht.

6. Filz nach Anspruch 5,
wobei der Nadelfilzprozess die Verwendung von 7.000 bis 9.000 Nadeln pro m² und 600 bis 800 Schlägen pro Minute vorsieht.

7. Filz nach einem der Ansprüche 1 bis 6,
wobei dieselben Filze in mehr oder weniger großen Stichen durchnäht werden.

8. Filz nach Anspruch 7,
wobei das Durchnähen ein Garn mit 100 % voranodisierten Acrylfasern vorsieht.

9. Filz nach Anspruch 7,
wobei das Durchnähen ein Garn mit 100 % Aramid-, Meta-Aramid- oder Para-Aramidfasern vorsieht.

10. Filz nach einem der Ansprüche 1 bis 9,
wobei der Filz eine Bindung umfasst, die aus einem Netz in mechanisch beständigem Material besteht.

11. Filz nach Anspruch 10,
wobei die Bindung innerhalb des Filzes enthalten ist.

12. Filz nach Anspruch 10,
wobei die Bindung auf eine der Filzflächen durch die üblichen Laminierungs- oder Schlichtungstechniken aufgebracht wird.

13. Filz nach Anspruch 1, mit Filzen nach einem der Ansprüche 2 bis 5, die miteinander nadelgefilzt sind.

14. Prozess zur Herstellung eines Filzes nach einem der Ansprüche 1 bis 6, wobei voranodisierte Acrylfasern in Flocken dem Kardierprozess ausgesetzt und in sich überlappende Schleier umgewandelt werden, die dann unter Verwendung von 5.000 bis 10.000 Nadeln pro m² und Ausführen von 400 - 800 Schlägen pro Minute nadelgefilzt werden; und die so erhaltenen Filze ihrerseits miteinander nadelgefilzt werden.

15. Prozess nach Anspruch 14,
wobei der Nadelfilzprozess unter Verwendung von 7.000 bis 9.000 Nadeln und 600 - 800 Schlägen pro Minute ausgeführt wird.

16. Verwendung der Filze nach einem der Ansprüche 1 bis 13 zur Herstellung von Isoliermaterialien.

17. Verwendung der Filze nach einem der Ansprüche 1 bis 13 zur Herstellung von Schutzbekleidung für Feuer und Wärme, zur Herstellung von Produkten für den Schutz von Materialien oder Anlagen vor Feuer, zur flammensicheren Textilpolsterung und Zubehör zum Ausstatten öffentlicher Bereiche.

18. Isoliermaterialien, die aus Filzen nach einem der Ansprüche 1 bis 13 hergestellt sind oder aus diesen bestehen.

19. Feuerfeste und hitzebeständige Bekleidungsstücke, Produkte, die zum Schutz von Materialien oder Anlagen vor Feuer verwendbar sind, flammensichere Textilpolsterungen und Zubehör zur Ausstattung öffentlicher Bereiche, Isoliermaterialien, die aus Filzen nach einem der Ansprüche 1 bis 13 hergestellt sind oder aus diesen bestehen.

20. Filze nach einem der Ansprüche 1 bis 13, wobei die voranodisierte Acrylfaser vom Typ LASTAN^{®}, PIROMEX^{®}, PANOX^{®}, PYRON^{®} ist oder aus deren Mischungen besteht.

## Revendications

1. Feutres comprenant des voiles se racouvrant, feutrés ensemble, consistant en fibres acryliques pré-anodisées.

2. Feutres selon la revendication 1, ayant une masse superficielle supérieure à 100 g/m².

3. Feutre selon la revendication 1, dans lequel le nombre de voiles est compris entre 6 et 11.

4. Feutre selon la revendication 3, dans lequel le nombre de voiles est compris entre 7 et 9.

5. Feutre selon les revendications 3 et 4, dans lequel les voiles subissent un processus de cardage et feutrage à l'aiguille qui prévoit de 5000 à 10000 aiguilles par m² et de 400 à 800 battements par minute.

6. Feutre selon la revendication 5 dans lequel le processus de feutrage à l'aiguille prévoit l'utilisation de 7000-9000 aiguilles par m² et 600-800 battements par minute.

7. Feutre selon les revendications 1-6, dans lequel les mêmes feutres sont piqués de points plus ou moins grands.

8. Feutre selon la revendication 7 dans lequel le piquage prévoit un fil comprenant 100% des fibres acryliques pré-anodisées.

9. Feutre selon la revendication 7 dans lequel le piquage prévoit un fil comprenant 100% de fibres aramidiques, méta-aramidiques, para-aramidiques.

10. Feutre selon les revendications 1-9 dans lequel ledit feutre comprend un tissage fait d'un filet en un matériau mécaniquement résistant.

11. Feutre selon la revendication 10, dans lequel ledit tissage est inclus à l'intérieur du feutre.

12. Feutre selon la revendication 10, dans lequel ledit tissage est appliqué sur l'une des surfaces du feutre par les techniques usuelles de stratification ou apprêt.

13. Feutre selon la revendication 1 comprenant des feutres selon les revendications 2-5 feutrés à l'aiguille ensemble.

14. Procédé pour la fabrication d'un feutre selon les revendications 1-6 dans lequel les fibres acryliques pré-anodisées, en flocons, subissent le processus de cardage et sont transformées en voiles se recouvrant qui sont alors feutrés en utilisant 5000-10000 aiguilles par m², en effectuant 400-800 battements par minute ; et les feutres ainsi obtenus sont à leur tour feutrés ensemble.

15. Procédé selon la revendication 14 dans lequel le procédé de feutrage à l'aiguille est effectué en utilisant 7000-9000 aiguilles et 600-800 battements par minute.

16. Utilisation des feutres selon les revendications 1-13 pour la fabrication de matériaux d'isolement.

17. Utilisation des feutres selon les revendications 1-13 pour la fabrication d'un tissu protecteur contre le feu et la chaleur, pour la fabrication de produits pour la protection des matériaux ou des plantes par rapport au feu, de capitonnages textiles ignifuges et d'accessoires pour l'ameublement des endroits réservés au public.

18. Matériaux isolants faits de ou comprenant des feutres selon les revendications 1-13.

19. Vêtements ignifuges et résistants à la chaleur, produits utiles pour la protection des matériaux ou plantes du feu, capitonnage textile ignifuge et accessoires pour l'ameublement des endroits réservés au public, matériaux isolants faits ou comprenant des feutres selon les revendications 1-13.

20. Feutres selon les revendications 1-13 dans lesquels la fibre acrylique pré-adonisée est du type LASTAN® PIROMEX®, PANOX®, PYRON® ou leurs mélanges.
